# EUROPEAN PATENT SPECIFICATION

(11) **EP 0 001 882 B1**
(45) Date of publication and mention of the grant of the patent: **09.12.1981**
(21) Application number: 78300393.2
(22) Date of filing: 18.09.1978
(51) Int. Cl.: H01H 1/02, H01B 1/22, H01H 13/10, H01H 13/70, H01H 35/00

(54) **Depressible contactless key for generating electric signals in an electronic keyboard**
Kontaktfreier Drücktaster zur Verwendung in einer elektronischen Tastatur
Touche à pression sans contact utilisable dans un clavier électronique

(30) Priority: 07.11.1977 IT 6948677
(43) Date of publication of application: 16.05.1979
(73) Proprietor: Ing. C. Olivetti & C., S.p.A., 10015 Ivrea (IT)
(72) Inventor: Varesio, Franco, Dr., Torino (IT)
(74) Representative: Pears, David Ashley

## Description

This invention relates to a depressible contactless key for generating electric signals in an electronic keyboard, e.g. for data processing equipment comprising a piezoconductive element formed of a matrix of insulating elastomeric material polymerized with a magnetic, metallic, conductive powder dispersed therein, the element having a flat shape with a pair of parallel large surfaces and extending between a pair of conductors, the key when depressed causing a compression spring to generate a force perpendicular to the said surfaces.

Elastomeric materials (rubbers) are known which are rendered conductive by adding materials such as carbon black or metal powders to the mix or composition. Some compositions and processes for producing conductive rubbers are given in the book: Conductive Rubbers and Plastics, by R. H. Norman - Elsevier, Amsterdam, London, New York, 1970.

Elements of conductive rubber are used as contact materials in some known types of keyboard. However, for application in keyboards, piezoconductive rubbers are more interesting, that is those rubbers which become conductive under the effect of applied pressure, because they allow keyboards without contacts exposed to oxidation to be obtained, inasmuch as contact takes place within the piezoconductive material.

Some piezoconductive elastomers are used for producing fixed contacts. In the known materials the piezoconductive effect disappears after a few thousand actuations of the elastomeric element, for which reason these materials are not suitable for use in keyboards.

A keyboard using such a piezoconductive rubber is known from the German Patent Specification 1,939,642, where the deformable piezoconductive element bridges two stationary contacts and is compressed through a spring urged member, upon depressing the key, to establish the electric connection of the two contacts. A keyboard with such a piezoconductive material is however not reliable for the reasons stated above.

The object of this invention is to provide a contactless keyboard wherein the piezoconductive element is very sensitive to the depression and release of the key and preserves its characteristics over a very high number of actuations.

This problem is solved by a key according to the invention, which is defined in the characterising part of claim 1.

The invention will be described in more detail, by way of example, with reference to the accompanying drawings in which:
Fig. 1 is a front view of an apparatus for preparing the elastomer to be used in a key according to the invention;
Fig. 2 shows a key employing the piezoconductive elastomer and embodying the invention;
Fig. 3 shows a detail of a keyboard employing keys according to the invention;
Fig. 4 is a graph relating to the key of Fig. 2;
Fig. 5 is a diagram of a measuring circuit used for the graph of Fig. 4.

Fig. 2 shows a key 10 which uses a patch 11 of piezoconductive elastomer and can be employed to replace a normal contact-type key as an input device for a data processing apparatus, with an interface towards semiconductor electronic circuits of high input impedance.

A housing 12 of the key rests on a printed circuit board 13 on which there is formed an island 14 with a diameter of 8 mm and connected to one end of the contact circuit of the key. The other end of this circuit is connected to another island 15 to which there is soldered a flexible metal plate 17 having a circular end 16 with a diameter of 8 mm.

The patch 11 of piezoconductive material, which has a diameter of 8 mm and a thickness of 0.6 mm, is fixed by means of conductive adhesive between the island 14 and the circular end 16 of the flexible plate 17.

On the end 16 there rests a spring 18 inserted in a recess 19 of a sliding shank 20 of the key 10, which bears a button 21. In the inoperative state, the spring 18 bears on the end 16 with a force sufficient to keep the button 21 raised.

When the button 21 is pressed, the force exerted is transmitted through the spring 18 and the end 16 of the flexible plate 17 to the patch 11 of piezoconductive rubber, reaching a value of about 10° when the button 21 strikes the top of the housway 12 of the key. Under the effect of the applied force, the patch 11 becomes conductive, ensuring a path of low resistivity between the islands 14 and 15.

For use of the key in a data entry keyboard, it is required that the patch 11 behave as a practically perfect insulator until the pressure applied reaches a predetermined value of about 80 g and to assume a low resistance when this pressure is exceeded, and then to reacquire the insulating properties on release of the key, presenting a certain hysteresis, but with a negligible delay. It is moreover essential that the patch preserves these characteristics for at least 100,000 operations of the same key, with a contact resistance always below 10,000 ohms.

According to the known literature (B. E. Springett: Conductivity of a system of metallic particles dispersed in an insulating medium - J. A. Phys., Vol. 44, No. 6, June 73, pp. 2925-26, and C. H. Kuist: Anisotropic conduction in elastomeric composites- Proc. 7 Am. Conn. Symposium, June 1974, pp. 203-209), on varying the percentage of metal powder in a matrix of insulating elastomer the conductivity of the whole shows a distinct transition from insulating material to conductive material for a well-defined percentage by volume (Vₘ) of metal powder close to 0.2 and dependent to a certain extent on the grain size and on the shape of the metal granules, presenting piezoconductive characteristics for percentages by volume of metal powders a little lower than Vₘ.

In particular in the article by C. H. Kuist, percentages of metal (nickel) powder by volume ranging between 0.08 and 0.18 are suggested for the piezoconductive rubbers.

It is known that the application of a magnetic field during the polymerization of rigid epoxy plastics materials containing metal powders (see the said book Conductive Rubbers and Plastics, page 82) brings a considerable increase in the conductivity of the whole in the direction of the magnetic field; it could therefore be expected from this that also with elastomers the application of a magnetic field during the polymerization would lead to a lowering of the transition percentage V m between the piezoconductive condition and the conductive condition in the preferred direction established by the magnetic field.

Surprisingly, it has been found that on dispersing nickel powders in a matrix of elastomeric binder, for example of the type Silastic E manufactured by Dow Corning, and maintaining the composition under the effect of a magnetic field during the polymerization of the binder, the rubber proves to be insulating in the absence of pressure even with percentages of powder between 15 and 27%, which greatly exceed the indicated limit values. On the other hand, the endurance of the piezoconductive characteristics improves decisively and passes from a few thousand operations of the key to several hundreds of thousands before irregularities of operation not tolerated by normal electronic utilization circuits are encountered.

It has also been found that on exceeding these percentages, the piezoconductive characteristics become worse again and that the optimum value is found for percentages around 21 %.

The preferred metal material is a nickel powder consisting of spherical grains and having the maximum hardness compatible with preservation of the magnetic characteristics. More particularly, good results have been obtained with a nickel powder known by the trade name of Alloy 79 GS, supplied by the Baudier Company, of Liancourt (France).

The powder consists of 93.94% of nickel, 3.5% of silicon, 1% of iron, 1.6% of boron and 0.05% of carbon and has a Rockwell C hardness of 18-22; the spherical granules have a diameter between 100 and 150,u.

A preferred composition of the piezoconductive elastomer is constituted by:
Silastic E silicone rubber from Dupont: by weight: 30 parts;
79 GS nickel powder from Baudier: 70 parts;
Silastic E hardener from Dupont: 3 parts.

Preparation of the piezoconductive elastomer requires careful mixing of the powder and silicone rubber, addition of the hardener, a first degassing of the mix under vacuum and casting in the mould followed by a second degassing under vacuum and introduction into the magnetizer, which applies a magnetic field with a direction perpendicular to the faces of the sheet during the polymerization of the binder.

The thickness of the sheet or film of piezoconductive elastomer may vary from 0.4 to 0.8 mm, preferred thickness being 0.6 mm.

The intensity of the magnetic field during the polymerization is not critical, provided that the field reaches an intensity of at least 500 oersteds. Above this value no appreciable variations are found in the results.

The apparatus used for preparing the elastomer is shown diagrammatically in Fig. 1, in which a mould 31 of non-magnetic material, in which the elastomer mix 36 is cast, is between two pole pieces 32 and 33 a magnetizer 37 which are interconnected by an external magnetic circuit (not shown). The magnetic flux is maintained throughout the time of polymerization of the elastomer by the current flowing in two windings 34 and 35. During the polymerization, the elastomer is kept at room temperature. Under these conditions, complete polymerization requires about 18 hours.

The time required for preparing the piezoconductive elastomeric material can be reduced to 10 minutes, still in a magnetic field, if the temperature of the mould 31 is brought to 100°C.

All the samples tested have exceeded the prescribed minimum life of 100,000 operations, with peaks of more than 1,000,000 operations.

Fig. 5 shows a simple circuit used for detecting the characteristics of the key of Fig. 2, comprising a DC voltage generator 41 producing 5 V and a 50 KQ limiting resistor 42 in series with the key 10.

Fig. 4 is a graph of the voltage drop detected across the terminals 43 and 44 of the resistor 42 as a function of the force F applied to the key. The phenomenon of hysteresis between actuation and release of the key is obvious from the graph.

An alternative embodiment of a keyboard employing the piezoconductive rubber is shown in Fig. 3.

In the keyboard 23, a single sheet 24 of piezoconductive material produced in a magnetic field is used, instead of individual patches of piezoconductive elastomer as in the key of Fig. 2. The sheet 24 is stuck by means of a conductive adhesive to islands 26 of a printed circuit board 25 which constitute one of the contact terminals of the keys 27.

A second, flexible, printed circuit board 28 is stuck by means of conductive adhesive on top of the sheet 24 of piezoconductive material at islands 29 in line with the islands 26. The islands 26 and 29 constitute contact terminals of the keys 27.

Springs 30, in combination with the movement of buttons 22, transmit the force applied to the buttons 22 to the piezoconductive sheet 24, causing locally the formation of passages of relatively low resistivity between the islands 26 and 29, while the material of the piezoconductive sheet 24 interposed between the keys 27 and not subjected to pressure maintains its insulating properties. The solution of Fig. 3, which is functionally equivalent to the modular solution of Fig. 2, is more convenient for producing keyboards with a large number of keys inasmuch as it drastically reduces the number of parts.

As regards the value of the actuating force applied to the keys, a maximum value of 100 g is required. Since it has been verified that the number of operations which can be obtained before the occurrence of irregularities increases with the value of the force applied, the maximum number of operations in keyboards employing the piezoconductive elastomer according to the invention can be further increased if, instead of the actuating force being obtained directly from the key, it is obtained from a lever system which presses on the piezoconductive rubber with a force higher than, for example double, that applied to the key, with a proportionally smaller stroke.

With this solution, it is possible to construct keys which simultaneously close a plurality of independent circuits by using a plurality of separate and insulated patches of piezoconductive material according to the invention or acting simultaneously on different points of the same sheet of piezoconductive material by means of actuating elements insulated from one another.

It is possible to make numerous variations in the solutions exemplified here as regards the type of elastomer and of magnetic conductive material, the form of the key, the level of modularity, that is the manner of grouping the keys, the actuating mechanism, and the production of contact between the piezoconductive material and the encoding circuit, without departing from the scope of the invention as claimed.

## Claims

1. A depressible contactless key for generating electric signals in an electronic keyboard, comprising a piezoconductive element (11) formed of a matrix of insulating elastomeric material polymerized with a magnetic, metallic, conductive powder dispersed therein, the element having a flat shape with a pair of parallel large surfaces and extending between a pair of conductors (14, 16), the key when depressed causing a compression spring (18) to generate a force perpendicular to said surfaces, characterised in that the piezoconductive element is rendered anisotropic, with prevailing piezoconductive properties in a direction perpendicular to the said large surfaces, by the action of a magnetic field applied thereto during the polymerization of the elastomeric material, the piezoconductive element having one of the large surfaces in contact with a first fixed conductor (14) of the said pair and the other large surface in contact with the other of the conductors (16), which is deformable or displaceable under the force generated by the compression spring (18) to compress the piezoconductive element in the said direction, whereby the electric connection of the conductors is very sensitive to the key depression.

2. A key according to claim 1, characterized in that the powder is a hard nickel powder formed of substantially spherical granules having a diameter between 100 and 150 It and a percentage in volume in the elastomeric material between 15% and 27%.

3. A key according to claim 1 or 2, characterized in that a plurality of the piezoconductive elements are provided, at least one of the pair of conductors being individual to each of the elements, the force being arranged to simultaneously compress the plurality of the elements.

4. A key according to claim 1 or 2, wherein the element is in form of a sheet, characterized in that the sheet has a constant thickness and is compressed by the said force on a predetermined limited area, the first one of the conductors being carried by a rigid printed circuit, the second conductor being carried by a flexible printed circuit, the sheet being sandwiched between the two printed circuits.

## Revendications

1. Une touche enfonçable sans contact pour engendrer des signaux électriques dans un clavier électronique, comprenant un élément piézo-conducteur (11) formé par une matrice en une matière élastomère isolante polymérisée dans laquelle une poudre métallique, magnétique, conductrice est dispersée, l'élément ayant une forme plate comportant une paire de grandes surfaces parallèles et s'étendant entre une paire de conducteurs (14, 16), la touche lorsqu'elle est enfoncée provoquant la production par un ressort de compression (18) d'une force perpendiculaire auxdites surfaces, caractérisée en ce que l'élément piézo-conducteur est rendu anisotrope avec des propriétés piézo- conductrices prédominantes dans une direction perpendiculaire auxdites grandes surfaces par l'action d'un champ magnétique qui lui est appliqué pendant la polymérisation de la matière élastomère, l'élément piézo-conducteur ayant l'une des grandes surfaces en contact avec un premier conducteur fixe (14) de ladite paire et l'autre grande surface en contact avec l'autre des conducteurs (16) qui est déformable ou déplaçable sous la force engendrée par le ressort de compression (18) pour comprimer l'élément piézo-conducteur dans ladite direction de telle sorte que la connexion électrique des conducteurs est très sensible à l'enfoncement de la touche.

2. Une touche selon la revendication 1, caractérisée en ce que la poudre est une poudre de nickel dur formée de granules approximativement sphériques ayant un diamètre compris entre 100 et 150 µm et un pourcentage en volume dans la matière élastomère compris entre 15% et 27%.

3. Une touche selon la revendication 1 ou 2, caractérisée en ce qu'il est prévu une série d'éléments piézo-conducteurs, au moins l'un des conducteurs de la paire de conducteurs étant propre à chacun des éléments, la force étant agencée de façon à comprimer simultanément la série d'éléments.

4. Une touche selon la revendication 1 ou 2 dans laquelle l'élément est sous forme d'une feuille, caractérisée en ce que la feuille a une épaisseur constante et est comprimée par ladite force sur une surface limitée prédéterminée, le premier des conducteurs étant porté par un circuit imprimé rigide, le second conducteur étant porté par un circuit imprimé flexible, la feuille étant emprisonnée entre les deux circuits imprimés.

## Patentansprüche

1. Niederdrückbare kontaktlose Taste zur Erzeugung elektrischer Signale in einer elektronischen Tastatur, enthaltend ein piezoleitendes Element (11), das aus eines Grundmasse eines isolierenden elastomeren Stoffes gebildet ist, der mit einem darin dispergierten magnetischen, metallischen, leitenden Pulver polymerisiert ist, und das eine flache Gestalt mit einem Paar paralleler großer Oberflächen aufweist und sich zwischen einem Paar von Leitern (14, 16) erstreckt, wobei die niedergedrückte Taste eine Druckfeder (18) veranlaßt, eine senkrecht zu den Oberflächen gerichtete Kraft zu erzeugen, dadurch gekennzeichnet, daß das piezoleitende Element durch die Wirkung eines während der Polymerisation des elastomeren Stoffes angelegten Magnetfelds mit vorherrschenden piezoleitenden Eigenschaften in einer senkrecht zu den genannten großen Oberflächen verlaufenden Richtung anisotrop gemacht ist und daß die eine große Oberfläche des piezoleitenden Elements mit einem ersten feststehenden Leiter (14) des Leiterpaares und die andere große Oberfläche des piezoleitenden Elements mit dem anderen Leiter (16) des Leiterpaares in Kontakt steht, der unter der von der Druckfeder (18) erzeugten Kraft deformierbar oder verschiebbar ist, um das piezoleitende Element in der genannten Richtung zusammenzudrücken, wodurch die elektrische Verbindung der Leiter gegenüber dem Niederdrücken der Taste sehr empfindlich ist.

2. Taste nach Anspruch 1, dadurch gekennzeichnet, daß das Pulver ein Hartnickelpulver aus im wesentlichen kugelförmigem Granulat mit einem Durchmesser zwischen 100 und 150 ,um und einem prozentualen Volumen im elastomeren Stoff zwischen 15 und 27% ist.

3. Taste nach Anspruch 1 oder 2, dadurch gekennzeichnet, daß eine Vielzahl der piezoleitenden Elemente vorgesehen ist, wenigstens eines der Leiterpaare jedem der Elemente einzeln zugehörig ist und die Kraft so arrangiert ist, daß die Vielzahl der Elemente gleichzeitig zusammengedrückt wird.

4. Taste nach Anspruch 1 oder 2, bei der das Element in Form einer dünnen Platte vorliegt, dadurch gekennzeichnet, daß die dünne Platte eine konstante Dicke hat und durch die Kraft in einem vorbestimmten begrenzten Bereich zusammengedrückt wird und daß der erste der Leiter von einer starren gedruckten Schaltung und der zweite der Leiter von einer flexiblen gedruckten Schaltung getragen wird und die dünne Platte zwischen die beiden gedruckten Schaltungen geschichtet ist.
